

Dec. 2, 1924.

1,517,892

K. R. DOUGLASS

LEATHER SUBSTITUTE AND METHOD OF MAKING THE SAME

Filed Nov. 22, 1919



K. R. Douglass, Inventor.

By his attorney. F. H. Squair.

## UNITED STATES PATENT OFFICE.

KENNETH R. DOUGLASS, OF WILMINGTON, DELAWARE, ASSIGNOR TO E. I. DU PONT DE NEMOURS & COMPANY, OF WILMINGTON, DELAWARE, A CORPORATION OF DELAWARE.

## LEATHER SUBSTITUTE AND METHOD OF MAKING THE SAME.

Application filed November 22, 1918. Serial No. 339,948.

To all whom it may concern:

Be it known that I, KENNETH R. DOUGLASS, a citizen of the United States, and a resident of Wilmington, in the county of New Castle and State of Delaware, have invented a certain new and useful Leather Substitute and Method of Making the Same, of which the following is a specification.

My invention relates to leather substitutes and has more particular reference to film-carrying textile fabrics adapted for use as substitutes for leather in furniture coverings, automobile upholstery, luggage, and so on, and also relates to methods of making such substitutes.

In the manufacture of materials of the character mentioned the desire is to produce an article that will be long-wearing, can be satisfactorily embossed, and will have the "feel" of leather. For proper embossing qualities and proper "feel" pyroxylin films are highly satisfactory and much used; but in using them it is common, and advisable, to add a softener, say castor oil, to insure flexibility. Yet, it is a matter of no small difficulty to get a proper and long-wearing attachment between a pyroxylin film sufficiently soft to give desired flexibility, and the fabric. I have devised a leather substitute which not only has a film with a properly flexible pyroxylin surface, whereby the substitute has the desired "feel" and embossing qualities and is long-wearing, but also has that film strongly and adequately attached to the fabric. And I have devised a method whereby such substitute can be manufactured readily and economically.

One object of my invention is to provide a leather substitute, in the character of a film-carrying textile fabric, of superior flexibility and surface and having its film strongly attached to its fabric.

Another object is to provide a leather substitute of the character indicated in which a lower film, that comprises a stratum of the entire film, is of rubber and, so, strongly attached to fabric, and in which an upper film is of pyroxylin and, so, well adapted for embossing and having a proper "feel," the lower and upper films being strongly attached to each other and united to form the entire film.

Another object is to provide a method whereby leather substitutes of the character

indicated can be made satisfactorily, expeditiously and relatively inexpensively.

To these and other ends, and also to improve generally upon substitutes and methods of the character indicated, my invention consists in the following matters hereinafter described and claimed.

The figure in the accompanying drawing is a conventional cross-sectional view of a leather substitute made in accordance with my invention.

In carrying out my invention I use two dissimilar films in building up the complete film on the fabric base, and place between the two a substance that adheres to both and firmly joints them together, i. e., a doubly-adherent substance. In this way I am enabled to use, for the film directly attached to the fabric, one which will adhere very firmly thereto, not having to consider the "feel" and so forth of its surface; and also I am enabled to use for the surface film a material having the surface and flexibility desired, not having to consider the ability of such surface film to adhere to the fabric. Thus the best materials for the particular qualities desired, i. e., adherence and flexibility for the lower film, and surface and flexibility for the upper, can be selected, and combined to give an article of superior wearing ability, and, at the same time, superior surface.

Stated more specifically, I proceed as follows:—I coat a fabric base with a rubber film that has the flexibility I desire and will adhere very firmly to the fabric, although since it is of rubber, it has not those qualities of surface which I desire. Then I coat the rubber film with linseed oil, preferably boiled to increase its drying properties, this oil having the ability to adhere very strongly both to rubber and to pyroxylin, and exemplifying a "doubly adherent" substance.

And, then, I apply a film of pyroxylin consisting, say, of several under coats of relatively heavy jelly and a less number of upper coats of relatively lighter jelly. This pyroxylin upper film gives the substitute a surface having the qualities of "feel," and satisfactory ability to be embossed, that I desire. And I can use in the pyroxylin film, preferably merely in the lower coats, that amount of softener needed to give desired flexibility, whatever might be the bad effect

of such an amount of softener on the ability of the pyroxylin to adhere to fabric.

In making a leather substitute embodying my invention, the procedure can satisfactorily be as follows (the various proportions given are by weight) :-

Using a textile fabric base, there is applied thereto a rubber compound dissolved in such an amount of solvent that it will spread evenly, said compound being such as will give a film that will remain flexible indefinitely; a sufficient number of coats, say five, being used to cover the fabric well, and each coat, preferably, being dried after its application, say five minutes at 80°-90° C. A proper compound is

|    | Parts.          |
|----|-----------------|
|    | Crude rubber    |
| 20 | Litharge        |
|    | Sulphur         |
|    | Carbon black    |
|    | Whiting         |
|    | Natural bitumen |

but these proportions may be widely varied. These materials are worked up with mixing rolls in the usual manner and the compound then dissolved in preferably either gasoline or 90% benzol, preferably two parts of solvent to one of compound being used, these proportions giving a desirable consistency for easy spreading.

After the rubber film is applied it is calendered, to give it a smooth surface, such a surface being desirable to insure against objectionable sinking in of the substance next to be applied.

Next, linseed oil, preferably boiled, is applied to the rubber film, in one or more coats, sufficient to give a good adherent film over the entire surface of the rubber film, the oil preferably being used with a solvent for the rubber; e. g. equal parts of oil and 90% benzol or gasoline being desirable and giving a relatively thin solution. Each coat is preferably dried for, for example, one hour or longer at 80° C. The oil used may vary from "stand" oil to the heaviest jelly which will absorb gasoline or benzol. As a dryer for the oil, lead or cobalt linoleate in an amount weighing, say, 2% of the weight of the oil may be used. Also, the use, with the oil, of gums and resins, such as mastic, rosin, copal or other resins commonly used in oil varnishes, in an amount weighing say 50%, more or less as desired, of the weight of the oil, materially lessens the time of drying, and such use is advisable.

Next, the material is cured, in the manner used in vulcanizing rubber, say for three hours at 120° C., the oil being dried during the vulcanizing.

Next, a coating of pyroxylin jelly of any desired heaviness, and containing a suitable softener, is applied to the oil-covered rub-

ber film. About five to ten coats may be used, each coat being dried say at 85° C. for a minute or two. These coats may be of any desired pyroxylin composition. Also, as previously pointed out, the amount of softener can be determined by the flexibility desired, not by the ability of the jelly to adhere to fabric. The following is a satisfactory jelly :-

| Parts.         | 75 |
|----------------|----|
| Solvent        | 88 |
| Nitrocellulose | 12 |
| Castor oil     | 18 |

The solvent may be, say, 60 parts of 90% benzol to 40 of ethyl acetate. To the jelly may be added such coloring matter as desired, say 15 parts, composed of 7½ parts castor oil and 7½ pigment.

Next there is applied, to complete the pyroxylin film, a clear top coating, consisting of one or two coats of a solution of, say, 10 parts of nitrocellulose to 90 parts of a solvent such as that given above, each coat being dried at, say, 85° C. for a minute or two.

Lastly, the finished material is dried for three or four days, or preferably a week, at about 20° C. to give full opportunity for the oil to dry.

The various rubber and pyroxylin coats may be applied in any suitable way, say by a standard "knife" coating machine, and the oil by, say, a "festooning" machine. It will be understood that, although I have given definite figures, proportions and so forth, I do not confine myself to them for, as will be evident, many departures from those figures can be made without departing from the invention.

I claim as my invention :

1. An article of manufacture comprising a fabric base carrying a series of superposed films thereon including a rubber film directly upon said base, a nitrocellulose film carried by said rubber film, and a doubly-adherent film, dissimilar to both said previously named films, between such two films.

2. An article of manufacture comprising a fabric base carrying a series of superposed films thereon including a rubber film directly upon said base, a nitrocellulose film carried by said rubber film, and a drying oil film therebetween.

3. An article of manufacture comprising a fabric base carrying a series of superposed films thereon including a rubber film directly upon said base, a nitrocellulose film carried by said rubber film, and a film of linseed oil therebetween.

4. An article of manufacture comprising a fabric base carrying a series of superposed films thereon including a rubber film directly upon said base, a nitrocellulose film carried by said rubber film and including a

softener, and a film of linseed oil therebetween.

5. An article of manufacture comprising a fabric base carrying a series of superposed films thereon, including a rubber film directly upon said base, a nitrocellulose film carried by said rubber film and including a softening oil, and a film of linseed oil therebetween.
- 10 6. An article of manufacture comprising a fabric base carrying a series of superposed films thereon including a rubber film directly upon said base, a nitrocellulose film carried by said rubber film, and a film of 15 linseed oil and resin therebetween.

7. An article of manufacture comprising a fabric base carrying a series of superposed films thereon, including a rubber film directly upon said base, a nitrocellulose film 20 carried by said rubber film and including a softener, and a film of linseed oil and resin therebetween.
8. An article of manufacture comprising a fabric base carrying a series of superposed films thereon, including a rubber film 25 directly upon said base, a nitrocellulose film

carried by said rubber film and including a softening oil, and a film of linseed oil and resin therebetween.

9. The method of manufacturing a coated 30 fabric which comprises, applying to the fabric a coating of dissolved rubber, removing the solvent of the rubber, calendering the rubber, applying a coating of linseed oil, vulcanizing the rubber and drying the oil, applying a coating of dissolved nitrocellulose, and removing the solvent of the nitrocellulose. 35

10. The method of manufacturing a coated fabric which comprises, applying to 40 the fabric a coating of dissolved rubber, removing the solvent of the rubber, calendering the rubber, applying a coating of linseed oil and rubber solvent, vulcanizing the rubber while removing the rubber solvent 45 and drying the oil, applying a coating of dissolved nitrocellulose, and removing the solvent of the nitrocellulose.

In testimony whereof I affix my signature.

KENNETH R. DOUGLASS.